

1

3,562,380

WEB-SPINNING FIBERS AND FILMS OF BENZIMIDAZO-BENZOPHENANTHROLINE POLYMERS  
Michael Dunay, Fanwood, and James A. Parker, Plainfield, N.J., assignors to Celanese Corporation, New York, N.Y., a corporation of Delaware  
No Drawing. Filed Mar. 21, 1969, Ser. No. 809,367  
Int. Cl. D01f 7/04

U.S. CL. 264—184

7 Claims

## ABSTRACT OF THE DISCLOSURE

Processes are provided for producing shaped articles such as fibers or films from sulfuric acid solutions of benzimidazo-benzophenanthroline polymers by extruding the solution into a coagulation medium which may be dimethylformamide, dimethylacetamide, N-methyl-2-pyrrolidone, or mixtures thereof. To improve physical properties the coagulated articles may be subsequently hot drawn.

## BACKGROUND OF THE INVENTION

### Field of the invention

This invention relates to a process for forming shaped articles from benzimidazo-benzophenanthroline polymers. This invention further relates to a process for forming filaments, fibers, films, and the like from bis(benzimidazo-benzophenanthroline) polymers which hereinafter may be referred to generally as BBB polymers.

### Description of the prior art

In recent years, new types of high temperature resistant polymers, such as the linear polybenzimidazoles (PBI), have attracted attention in connection with the fabrication of articles such as re-entry parachutes for space vehicles, high temperature insulating materials, and the like. As an outgrowth of this, polymers of the benzimidazo-benzophenanthroline type, and particularly the poly(bisbenzimidazo-benzophenanthroline) type (BBB), made as described, for example, in an earlier copending application, Ser. No. 657,868, filed Aug. 2, 1967, and assigned to the assignee of the present application, have been found to give particularly useful products in this connection.

As described in the aforementioned copending application Ser. No. 657,868, fibers and other shaped articles of satisfactory properties can be made from BBB type polymers by solution spinning a dope containing the BBB polymer dissolved in sulfuric acid solvent into an aqueous dilute sulfuric acid coagulation bath. After such wet spinning, the resulting precursor (as spun) fibers or other shaped articles are normally washed thoroughly in a dilute alkaline bath in order to neutralize and remove excess sulfuric acid, thereafter washed with water, and then hot drawn to improve their physical characteristics, e.g., tenacity, elongation, etc.

Disadvantages, however, normally associated with the above described wet spinning process include the necessity of using the alkaline wash bath to neutralize and remove excess sulfuric acid, and the apparent inability of the process to produce high, e.g., 100 or higher, denier filaments or fibers without incurring unwanted voids in the filament or fiber structure.

2

The search has continued, therefore, for alternative processes for forming shaped articles from the benzimidazo-benzophenanthroline polymers. The present invention was made as a result of that search.

### SUMMARY OF THE INVENTION

Accordingly, an object of the present invention is to provide processes for forming shaped articles, such as filaments and fibers, from benzimidazo-benzophenanthroline polymers.

Another object of the present invention is to provide a wet spinning process for producing shaped articles from sulfuric acid solutions, i.e., dopes, of bisbenzimidazo-benzophenanthroline (BBB) polymers, which process avoids or substantially alleviates the disadvantages of such processes heretofore described.

A further object is the provision of a wet spinning process for sulfuric acid solutions of BBB polymers which employs novel coagulating baths in the system, which process does not require subsequent acid neutralizing baths, and which can produce high denier BBB fibers that are substantially void-free.

Other and further objects of the invention will become apparent from the following more detailed description.

In accordance with the present invention, shaped articles such as filaments, fibers and films are formed from benzimidazo-benzophenanthroline polymers by preparing a dope or solution of the polymer in an acid solvent such as concentrated sulfuric acid, and extruding the acid dope or solution into a coagulation medium consisting essentially of an amide which can be dimethylformamide, dimethylacetamide, N-methyl-2-pyrrolidone, or mixtures thereof.

Preferably, the coagulation medium consists essentially of dimethylacetamide.

Further, there is normally no need for any subsequent acid neutralizing bath for the amide coagulation medium concurrently neutralizes the acid solvent.

After the concurrent coagulation and neutralization, the shaped articles such as fibers or films can be washed with water to remove any amide, and hot drawn to improve physical properties. The articles obtained thereby are essentially void-free and may have a denier of 100 or higher.

### DESCRIPTION OF PREFERRED EMBODIMENTS

#### The starting polymer

The present invention is generally applicable to benzimidazo-benzophenanthroline polymers, and more preferably, to poly(bisbenzimidazo-benzophenanthroline).

As is now otherwise known in the art, these BBB type polymers are made by mixing and condensing (1) at least one organic tetraamine having the structural formula



wherein R is a monocyclic or bicyclic aromatic or cycloaliphatic tetravalent hydrocarbon radical and wherein each of the four amino groups is attached directly to a carbon atom of a ring of said aromatic or cycloaliphatic radical in a position which is ortho or peri (in the case of a bicyclic radical) to another carbon atom to which a second amino group is also directly attached; with (2)

at least one tetracarboxylic acid (which also may be in the form of a corresponding anhydride) having the structural formula



wherein R' is a tetravalent radical containing at least 2 carbon atoms and wherein no more than 2 carboxyl or carbonyl groups of said acid or anhydride are attached to any one carbon atom of said tetravalent radical.

Preferably, the tetraamine and the tetracarboxylic acid are reacted in substantially equal molar quantities.

The polymer used herein may have an inherent viscosity of at least .3 and, preferably about 1.0 to 5.0, and most preferably about 2.0 to 3.0.

The inherent viscosity as used herein as measured at 25° C. using a concentration of .4 g. of the polymer in 100 ml. of 97% H<sub>2</sub>SO<sub>4</sub>.

Nonlimiting examples of the tetraamine monomers which may be used individually or in mutual admixture in forming the desired polymers are: 3,3'-diaminobenzidine; bis (3,4-diamino phenyl) methane; 1,2-bis (3,4-diamino phenyl) ethane; 2,2-bis (3,4-diamino phenyl) propane; bis (3,4-diamino phenyl) ether; bis (3,4-diamino phenyl) sulfide; bis (3,4-diamino phenyl) sulfone; 1,2,4,5-tetraamino benzene; 2,3,6,7-tetraamino naphthalene; and the corresponding ring hydrogenated tetraamines.

Nonlimiting examples of the tetracarboxylic acids include:

pyromellitic acid;  
2,3,6,7-naphthalene tetracarboxylic acid;  
3,3',4,4'-diphenyl tetracarboxylic acid;  
1,4,5,8-naphthalene tetracarboxylic acid;  
2,2',3,3'-diphenyl tetracarboxylic acid;  
2,2-bis(3,4-dicarboxyphenyl) propane acid;  
bis (3,4-dicarboxyphenyl) sulfone acid;  
3,4,9,10-perylene tetracarboxylic acid;  
bis(3,4-dicarboxyphenyl) ether;  
ethylene tetracarboxylic acid;  
naphthalene 1,2,4,5-tetracarboxylic acid;  
decahydronaphthalene-1,4,5,8-tetracarboxylic acid;  
4,8-dimethyl-1,2,3,5,6,7-hexahydronaphthalene-1,2,5,6-tetracarboxylic acid;  
2,6-dichloronaphthalene-1,4,5,8-tetracarboxylic acid;  
2,7-dichloronaphthalene-1,4,5,8-tetracarboxylic acid;  
2,3,6,7-tetrachloronaphthalene-1,4,5,8-tetracarboxylic acid;  
phenanthrene-1,8,9,10-tetracarboxylic acid;  
cyclopentane-1,2,3,4-tetracarboxylic acid;  
pyrrolidine-2,3,4,5-tetracarboxylic acid;  
pyrazine-2,3,5,6-tetracarboxylic acid;  
2,2-bis (2,3-dicarboxyphenyl) propane acid;  
1,1-bis (2,3-dicarboxyphenyl) ethane acid;  
1,1-bis (3,4-dicarboxyphenyl) ethane acid;  
bis (2,3-dicarboxyphenyl) methane acid;  
bis (3,4-dicarboxyphenyl) methane acid;  
bis (3,4-dicarboxyphenyl) sulfone acid;  
benzene-1,2,3,4-tetracarboxylic acid;  
1,2,3,4-butane tetracarboxylic acid;  
thiophene-2,3,4,5-tetracarboxylic acid;  
and similar acids, as well as the anhydrides of such acids.

In a preferred embodiment, the present invention is directed to fibers formed from poly(bisbenzimidazobenzophenanthroline), i.e., BBB polymers. Such polymers are formed from 1,4,5,8-naphthalene tetracarboxylic acid and 3,3'-diamino benzidine according to the following equation:



A preferred method of preparing BBB polymers includes effecting the polymerization in polyphosphoric acid (PPA) where the reaction according to Equation A occurs and can produce a fully cyclized polymer.

15 Use of polyphosphoric acid as the solvent permits reactions to be carried out over a wide range of temperatures, e.g., 80° C. to 300° C., more preferably 100° C. to 250° C., and most preferably, 150° C. to 225° C.

The polyphosphoric acid preferably employed has a

20 P<sub>2</sub>O<sub>5</sub> equivalent of about 82% to 84%, by weight, which is a solution of approximately 5% to 20% ortho- and pyrophosphoric acids mixed with various polyphosphoric acids, mostly trimers, tetramers, pentamers and hexamers.

25 The tetraamines and tetracarboxylic acid or corresponding dianhydride may also be reacted in an organic liquid which is solvent for at least one of the reactants, and is inert to the reactants, preferably under anhydrous conditions, at a temperature below 125° C., preferably at below 100° C.

30 To cyclize completely the polymer, subsequent high temperature heating may be required in the above described reaction or polymerization process.

Both the reaction temperature and the reaction period used significantly affects the degree of polymerization.

35 Generally, reaction periods can range from about 0.5 to 100 hours, typically 10 to 50 hours, at the above mentioned reaction temperatures. Higher reaction temperatures tend to result in polymer products having higher inherent viscosity than polymers produced at lower temperatures in comparable reaction times.

40 The manner in which the BBB polymer is formed or polymerized is not a part of the present invention. Thus, any method in addition to those described above may be used by those skilled in the art.

45 Wet spinning

The polymers of the type just described can be formed into fibers and other shaped articles by extruding a solution of the polymer in sulfuric acid through an opening 50 of predetermined shape into a coagulation medium or bath consisting essentially of an amide such as dimethylacetamide, which results in a coagulated material of a desired cross-section.

BBB solutions or dopes can be prepared by dissolving 55 sufficient polymer in sulfuric acid to yield a final solution suitable for spinning or extrusion which contains about 2% to 15%, preferably about 3% to 10%, and most preferably about 4% to 6%, by weight, of polymer based on the total weight of the solution.

60 The sulfuric acid employed should be at least 92 equivalent weight percent sulfuric acid, and is preferably from 97 to 100 equivalent weight percent sulfuric acid.

Further, the spinning or casting dopes may contain small amounts, e.g., about .001 to 1% by weight, of 65 various stabilizing additives and the like.

As stated above, the polymer spinning solution is then extruded into a coagulation bath consisting essentially of an amide such as dimethylacetamide, which is preferred. Other suitable amides include dimethylformamide, N-methyl-2-pyrrolidone, and mixtures thereof.

The coagulation bath may also contain minor amounts e.g., .001 to 10 weight percent of well known additives, e.g., other components which are acid acceptors such as aliphatic and aromatic amines, as well as inert species, 75 e.g., aliphatic and aromatic hydrocarbons, which would

not substantially affect the concurrent coagulation and neutralization.

As stated, the coagulation bath also serves to neutralize the acid in the spun fibers and must therefore be replaced with fresh amide on a batch wise, continuous, or semi-continuous basis as is well known to those skilled in the art. Preferably, a continuous stream of fresh amide is added to the coagulating bath with a corresponding removal of the spent amide.

The coagulating bath may be adjusted so that bath temperatures and residence times effect a reasonable speed in the coagulation of the shaped articles. Generally, bath temperatures between about 20° C. and the boiling point of the amide, and preferably between 25° C. and 100° C., and residence times of a few seconds to several minutes, e.g., preferably about 5 seconds to 5 minutes, and more preferably about 10 to 20 seconds, are used.

After such wet spinning, the resulting precursor (as spun) fibers or other shaped articles may be washed with water in order to remove excess amide and neutralized acid.

The water washing medium is usually maintained at a temperature of about 25° C. to 90° C., and preferably at about 50° C. to 80° C., and is usually contained in a bath through which the shaped articles are passed subsequent to their passage through the coagulation bath, as in a continuous process.

To improve physical properties, the fibers or other shaped articles may be hot drawn at temperatures of at least about 250° C., e.g., temperatures of about 250° C. to 700° C.

Preferably, the fibers or other shaped articles are hot drawn while still wet, e.g., contain from about 50 and up to 500 percent by weight of water, due to the water wash. Surprisingly, this gives the advantage of being able to draw at lower temperatures, e.g., about 250° C. to 350° C., and preferably about 260° C. to 280° C., versus the higher temperatures, e.g., 500° C. to 600° C., which may be required when substantially dry fibers are hot drawn.

The heat source for the hot drawing may be a heated drawing shoe, a heated rod or pin, a muffle furnace, or the like as is conventionally used and well known in the art.

The shaped articles may be hot drawn at draw ratios of about 1.1 to about 3.0, and preferably between about 1.2 and about 1.5. The term "draw ratio" as used herein has the conventional meaning as used in the art and is the ratio of the peripheral speed, in units of length per unit time, of the wind-up or take-up roll to that of the feed or delivery roll in the drawing system.

The present invention is further illustrated by the following examples which produce strong and void-free BBB fibers. All parts and percentages in the examples, as well as in the specification and claims, are by weight unless otherwise indicated.

#### EXAMPLE I

The BBB polymer used is a condensation product of 1,4,5,8-naphthalene tetracarboxylic acid and 3,3'-diaminobenzidine having an inherent viscosity of about 2.6. For use in the illustrative operation, this polymer is dissolved in 97% sulfuric acid to form a spinning solution containing about 5% dissolved polymer and characterized by a solution viscosity of 2100 poises at 60° C.

This solution is charged into a reservoir from whence it is extruded under 65 p.s.i.g. pressure through a conventional spinneret immersed in a coagulation bath, spinning at a rate of about 2 m./min.

The spinneret is a one-fil, 200-micron jet, i.e., a spinneret having an orifice of 200-micron diameter, though other spinnerets may, of course, be used similarly.

The coagulation bath used is 100% dimethylacetamide, and is at a temperature of about 25° C., with a fiber residence time in the coagulation bath of about 15 seconds.

The resulting wet spun fibers pass from the coagulation bath to a water wash which is maintained at a tem-

perature of about 80° C. with a residence time of about 5 seconds in the wash bath.

From the wash bath the washed fibers while still wet pass over a heated drawing shoe maintained at a temperature of 270° C., with a shoe residence time of about 2 seconds. A draw ratio of about 1.5 is maintained.

The resulting BBB fibers are of good quality, i.e., are strong and void-free.

#### EXAMPLE II

10 Example I is repeated with the exception that a coagulation bath of dimethylformamide is substituted for the coagulation bath of dimethylacetamide to produce BBB fibers of good quality.

15 EXPLANATION III

Example I is repeated with the exception that a coagulation bath of N - methyl - 2 - pyrrolidone is substituted for the coagulation bath of dimethylacetamide to produce BBB fibers of good quality.

20 While the invention has been described in preferred embodiments, variations and changes may be made therein without departing from the spirit of the invention.

We claim:

1. An improved process for forming fibers or films of 25 benzimidazo - benzophenanthroline polymer which process comprises

(a) forming an acid spinning dope containing between 30 about 2% and 15% of the polymer dissolved in sulfuric acid solvent having an H<sub>2</sub>SO<sub>4</sub> content of at least about 92%,

35 (b) extruding the resulting dope into a coagulation medium consisting essentially of an amide selected from the group consisting of dimethylformamide, dimethylacetamide, N - methyl - 2 - pyrrolidone, and mixtures thereof maintained at a temperature between about 25° C. and 100° C., and thereafter,

(c) recovering the coagulated material.

2. A process according to claim 1 wherein the coagulation medium consists essentially of dimethylacetamide.

40 3. A process according to claim 1 which further comprises

(i) washing the resulting coagulated material with water,

45 (ii) drawing the washed material at a temperature above about 250° C. and thereafter

(iii) recovering the drawn material.

4. An improved process for forming fibers or films from an acid dope containing bis(benzimidazo-benzophenanthroline) polymer dissolved in sulfuric acid solvent having an H<sub>2</sub>SO<sub>4</sub> content of at least 92%, the dope comprising between about 3% and 10% dissolved polymer, which process comprises

50 (a) extruding the dope through an orifice into a coagulation medium consisting essentially of an amide selected from the group consisting of dimethylformamide, dimethylacetamide, and N - methyl - 2 - pyrrolidone, at a temperature between about 25° C. and 100° C.,

55 (b) washing the resulting coagulated material with water,

60 (c) drawing the washed material at a draw ratio between about 1.1 and 3.0, and thereafter

(d) recovering the resulting material.

5. A process according to claim 4 wherein the drawing is done at a draw ratio between about 1.2 and about 1.5 and at a temperature between about 250° C. and 700° C.

65 6. A process according to claim 5 wherein the bath consists essentially of dimethylacetamide and is at a temperature between about 250 C. and 70° C.

70 7. An improved process for forming fibers of bis(benzimidazo-benzophenanthroline) polymer, which process comprises,

(a) forming a dope of the polymer in sulfuric acid solvent having an H<sub>2</sub>SO<sub>4</sub> content of at least 97%, the

- resulting dope comprising between about 4% to 6% dissolved polymer,  
 (b) spinning the resulting dope into a coagulation medium consisting essentially of dimethylacetamide at a temperature between about 25° C. and 70° C.,  
 (c) washing the resulting coagulated fibers with water,  
 (d) drawing the washed fibers while still wet, at a draw ratio between about 1.1 and about 3.0 and at a temperature between about 250° C. and 350° C., and  
 (e) thereafter recovering the resulting drawn fibers.

## OTHER REFERENCES

5 Gloor: "Fiber Formation and Drawing of Poly (bis-benzimidazo-benzophenanthroline)" from "Fiber Spinning and Drawing," edited by Coplan, Interscience Publishers, 1967 pp. 151-163.

5 "Symposium Focuses on Heat-Resistant Fibers," Chemical & Engineering News, Sept. 23, 1968, pp. 40-41.

10 JULIUS FROME, Primary Examiner

10 H. MINTZ, Assistant Examiner

## U.S. Cl. X.R.

264—203, 210; 260—47, 78

3,414,543 12/1968 Paufler ----- 260—47  
 3,441,640 4/1969 Santangelo ----- 264—203 15

## References Cited

## UNITED STATES PATENTS

UNITED STATES PATENT OFFICE  
CERTIFICATE OF CORRECTION

Patent No. 3,562,380 Dated February 9, 1971

Inventor(s) Michael Dunay and James A. Parker

It is certified that error appears in the above-identified patent and that said Letters Patent are hereby corrected as shown below:

In column 2, line 10, delete "objert" and insert "object"

In column 5, line 49, delete "drawiig" and insert "drawing"

In column 6, line 70, delete "250 C." and insert "25°C."

Signed and sealed this 22nd day of June 1971.

(SEAL)

Attest:

EDWARD M.FLETCHER, JR.  
Attesting Officer

WILLIAM E. SCHUYLER, JR.  
Commissioner of Patents